

May 8, 1934.

T. E. RICHARDS

1,957,850

PRINTING PLATE AND METHOD OF MAKING THE SAME

Filed Oct. 20, 1927

— fig. 1.



— fig. 2.



— fig. 3.



INVENTOR.

Thomas Ernest Richards  
BY  
F. P. Hayfield  
ATTORNEY.

## UNITED STATES PATENT OFFICE

1,957,850

PRINTING PLATE AND METHOD OF  
MAKING THE SAME

Thomas Ernest Richards, Auckland, New Zealand

Application October 20, 1927, Serial No. 227,623  
In New Zealand November 22, 1926

18 Claims. (Cl. 41—41.5)

This invention relates to lithographic printing plates and to the method of preparing the same, especially when prepared photographically; and has for its object the production of plates which will be superior to the plates heretofore in use with respect to cost and rapidity of preparation, durability, speed at which the plates may be run in the printing machines and quality of the work produced. This application has been divided; 5 claims for the method of making printing plates photographically appearing in my co-pending application, Serial No. 368,424, filed June 4, 1929.

The present invention is particularly adapted to the production of planographic plates for offset printing purposes, especially for newspaper work, but it is nevertheless contemplated applying the invention to the preparation of lithographic plates of any type.

By the present invention, one is enabled to produce a planographic printing plate having a very strong, distinct and durable image which may be put in an offset printing press, for example, and copies taken therefrom at a higher rate of speed and in greater quantity than have heretofore been practicable in this class of work. The image is defined by a coating material which is made hard and firmly united with the plate by partial penetration of the metal in a manner more specifically pointed out hereinafter.

30 The invention accordingly comprises the several steps and relation and order of one or more of such steps with respect to each of the others, and the printing plate possessing the features, properties, and the relation of elements, which are exemplified in the following detailed disclosure, and the scope of the application of which will be indicated in the claims.

For a fuller understanding of the nature and objects of the invention, reference should be had 40 to the following detailed description taken in connection with the accompanying drawing, in which:

Fig. 1 is an enlarged cross section showing schematically a grained plate having an image-receiving film.

Fig. 2 shows a plate of the character shown in Fig. 1 having a developed image to which is applied a coating containing an agent of durable character in accordance with the invention; and 50 Fig. 3 is a similar view showing the plate with the image film removed to yield a lithographic printing plate of the present invention.

Referring now to the drawing, 10 denotes a grained metallic plate of any suitable ink-repellent metal, for example, zinc or aluminum, to

which is applied a film 11 adapted to take an image, for example, a light sensitive film for receiving an image photographically. When an image has been formed or developed by removing portions of the film from the plate, there remain 60 upstanding portions as indicated at 12 in Fig. 2, about which the image-reproducing material is applied. To this end, a coating 13 containing an agent of durable character is applied evenly over the plate. The plate when finally prepared in accordance with the process of the present invention, has the image-receiving film removed and the coating hardened and made firmly adherently to the plate. This coating represents the image form to be reproduced by planographic printing 70 and stands alone on the finished plate as indicated in Fig. 3, the height shown being greatly exaggerated. The bonding of this coating to the metal by partial penetration thereof is indicated at 14.

When producing lithographic plates photographically, there are in general four main steps to be followed, namely, (1) producing a photographic image upon a sensitized metal printing plate by exposing a photographic film thereon, 80 (2) dissolving off the unexposed sensitive substance, (3) applying to the plate a coating material capable of taking and holding a desired image form and of absorbing printer's ink, (4) and finally developing the image on the plate according to any known or suitable method of removing the exposed or relatively exposed portions 85 of the sensitized substances.

In the practice of the present invention, the coating material is made to have metal penetrating and adhering properties, and is so applied to the plate and the whole so treated by means of heat that the coating becomes highly adherent and relatively hard whereby clear sharply defined images result and the plate produced capable of giving a relatively large number of impressions without sign of deterioration. In accomplishing this effect, a coating material is employed containing a body-giving agent of durable character, an ink-absorbing substance and a metal penetrating agent, which is applied to the plate about the developed image and heated in two stages, in the first of which the coating material is made closely adherent to the plate whereby the developed image substance may be removed in a 100 clean and efficient manner, while in the second the coating is hardened and firmly bonded with the plate.

Certain other steps which will be hereinafter described with reference to an illustrative exam- 110

ple of the invention are of minor importance and, except as hereafter noted and pointed out in the appended claims, are common practice and comprise no part of the invention.

- 5 The following procedure is an illustrative example of a specific method by which the present invention is carried out:

10 A grained metal lithographic plate is first prepared by rinsing a suitable metal plate, for example one of aluminum, in a ten percent solution of nitric acid and then thoroughly washed. The plate is then coated with a sensitized solution, for example, the following:

|                                 |              |
|---------------------------------|--------------|
| 15 Fish glue-----               | 16 ozs.      |
| Water -----                     | 36 ozs.      |
| Ammonium bichromate -----       | 1 1/2 ozs.   |
| Ferric ammonia citrate-----     | 1/2 oz.      |
| Strong solution of ammonia----- | 1 1/2 drams. |

- 20 On this sensitized plate an exposure is made from a half-tone screened or line positive. (Obviously, a negative may be employed if it is desired to make prints having their lights and shadows reversed as compared with the original.)

- 25 The image is then developed by washing the plate with water, which dissolves off the unexposed portions of the sensitized glue, leaving a negative image on the plate. The plate is next dried and afterwards coated with the penetrating ink-

- 30 absorbing substance, as referred to above, which is a liquid or plastic material prepared with a suitable solvent or vehicle and a rugged material, such as asphaltum, to give it body and durability. The following formula for the coating material

- 35 has been found to give satisfactory results: one gallon of pure turpentine (the solvent) is mixed with one pound of asphaltum (the body-giving material) and the mixture brought to the boiling point. This mixture is then combined with

- 40 a second mixture consisting of one-half pound of transfer ink dissolved by heating in one quart of turpentine. To this is added a third or liquid mixture comprising one dram of a preparation consisting of oleic acid and an essential oil, and

- 45 one dram of substantially pure oleic acid oil. The preparation of oleic acid and an essential oil preferred is that now sold on the open market under the tradename "Elbagreen oil". This mixture has the property of penetrating and adhering to

- 50 the plate, and being of a greasy nature, has affinity for printer's ink, as is well known in the art. The addition of the transfer ink to this mixture increases the affinity of the coating material.

- 55 The plate is coated with such material in any convenient uniform manner, for example by the whirling method, and then given the first heating, which is to a relatively moderate temperature, for example to 112° F. This temperature is sufficiently high to soften the coating but is not such as to crack the insoluble glue or film remaining on the plate, hence in general the figure given should not be exceeded. At this stage, the plate is entirely covered with some sort of material, the unexposed portions of the plate, which were washed clean by water being covered by the metal penetrating coating material, while the exposed portions are still protected by the insoluble glue or film.

- 70 The plate is now finally developed, which is accomplished by immersing it in water, so that the surplus coating material overlying the remaining glue may be brushed away. It is then placed in a ten percent solution of phosphoric acid, so that the undeveloped glue or film may

be dissolved or otherwise removed; after this the plate is washed with water; immersed in a ten percent solution of nitric acid for about twenty seconds; again washed with water; and immersed finally for one minute in a ten percent solution of phosphoric acid. 80

The plate is now washed, brushed and dried and then given its second heating which is to a relatively high temperature, for example to a temperature of from 250° to 260° F. This heating is such as materially to assist the coating material to penetrate the surface of the plate and become hard and thoroughly bonded with the metal of the plate in a firm and durable manner. It is beneficial to continue such heating for several minutes to give ample time for accomplishing this effect. Care, however, should be exercised not to continue the second heating for such a length of time or at such intensity as to cause injury to the plate. 85 90 95

When the plate has become cooled, it may be coated with a solution of gum arabic and dried. The plate is now ready to be put in the printing press and run.

The image thus provided on the plate is a tough, 100 closely adhering coating of ink-absorbing nature, the remainder of the plate being clean. The image is very durable, absorbs ink readily, and gives good depth of color. In consequence the plate can be run at high speed and will produce 105 more good prints than have heretofore been obtainable.

It will be understood that the particular ingredients mentioned in the foregoing description are not of the essence of the invention, and that some of the operations described, although practically necessary, are of a routine nature and well known in the art. The invention is not limited to the particular procedure described, except as defined in the following claims. The term "film" is used throughout in its generic sense, to designate any image-receiving substance. 110 115 120

I claim as my invention:

1. A lithographic printing plate which consists of an ink-repellent metallic sheet having a grained surface, and a coating comprising asphaltum, an ink-absorbing substance, oleic acid and an essential oil applied to said plate, shaped to have the configuration of a desired image and 120 125 adhering closely to the plate, said coating having the property of being relatively hard and bonded to said plate with partial penetration of the metal.

2. A lithographic printing plate, which consists of a sheet of ink-repellent metal having a grained surface initially coated with a film, an image on said surface formed from said film, there being bare metal exposed about the image-form, and a coating comprising asphaltum, a transfer-ink substance, oleic acid and an essential oil applied to said bare metal, said coating adhering closely to the metal plate, and having the property of penetrating the metal and of softening when heated and when cold of being relatively 130 135 140 hard and bonded to said plate.

3. The method of preparing lithographic printing plates, which comprises preparing a grained metallic plate having an image-form thereon, applying a coating material to said plate about 145 said image-form, said coating having metal penetrating properties, moderately heating said plate, removing the image-form, and then heating to a relatively high temperature.

4. The method of preparing lithographic print- 150

- ing plates, which comprises preparing a grained metallic plate having an image-form thereon, applying a coating material containing an agent of a durable character and a metal-penetrating oily agent to said plate about said image-form, moderately heating said plate, removing the material of said image-form, and then heating said plate to a relatively high temperature. 5. The method of preparing lithographic printing plates, which comprises preparing a grained metallic plate having an image-form thereon, applying a coating material containing asphaltum and a metal-penetrating oily agent to said plate about said image form, moderately heating said plate, removing said image-form, and then heating to a relatively high temperature. 6. The method of preparing lithographic printing plates, which comprises preparing a grained metallic plate having an image-form thereon, applying a coating material to said plate containing an agent of a durable character, an ink-absorbing substance and a metal-penetrating oily agent, moderately heating said plate, removing said image-form, and then heating said plate to a temperature such as to assist in causing said coating material to penetrate the metal of said plate and to become hard and firmly bonded therewith without injury to said plate. 7. The method of preparing lithographic printing plates, which comprises preparing a grained metallic plate having an image-form thereon, applying a coating material to said plate containing asphaltum, an ink-absorbing substance and a metal-penetrating oily agent, moderately heating said plate, removing said image-form, and then heating said plate to a relatively high temperature such as to assist in causing said coating material to penetrate the metal of said plate and to become hard and firmly bonded thereto without injury to said plate. 8. The method of preparing lithographic printing plates, which comprises preparing a grained metallic plate having an image-form thereon, applying a coating material to said plate containing asphaltum, a transfer-ink substance, oleic acid and an essential oil, heating said plate to a moderate temperature, removing said image-form and then heating said plate to a relatively high temperature such as to assist in causing the coating material to penetrate the metal and to become hard and firmly bonded thereto without injury to the plate. 9. The method of preparing lithographic printing plates, which comprises preparing a grained aluminum plate having an image-form thereon, applying a coating material containing asphaltum, a transfer-ink substance, oleic acid and an essential oil, heating said plates to a temperature approximating 112 degrees F., then removing the image-form, and thereafter heating said plate to a temperature approximately in the neighborhood of from 250 to 260 degrees F. 10. A planographic metallic printing plate having a finely grained surface and printing image areas thereon, said image areas being coated with a hardened bituminous ink-receiving material having its under-portions impregnated in the metal of the plate and constituting an embedded printing image. 11. A planographic metallic printing plate having a finely grained surface and printing image areas thereon, said image areas being coated with a hardened ink-receiving material containing an asphaltum base penetrating and firmly impregnated in said metal plate. 12. A planographic metallic printing plate having a surface thereof penetrable by an asphaltum composition, said surface being grained to take water and having delineated areas of a permanent character corresponding to an image to be printed, said areas being covered by hardened asphaltum base material impregnated in said plate. 13. A planographic metallic printing plate having a finely grained surface and permanent delineated areas thereon corresponding to an image to be printed, said areas being impregnated by ink-receiving material containing a hardened asphaltum base. 14. A planographic metallic printing plate having a finely grained surface and having thereon permanent delineated areas corresponding to an image to be printed, said areas being impregnated by ink-receiving portions of hardened asphaltum base material imbedded in the surface of the plate. 15. A planographic metallic printing plate having a finely grained surface capable of receiving water and permanent delineated areas thereon corresponding to an image to be printed, said areas being coated with hardened bituminous ink-receiving material having portions impregnated in said metallic plate, and constituting an embedded printing image. 16. A metal printing plate having ink-receiving portions of hardened asphaltum base material penetrating and embedded in the interstices of said plate. 17. A planographic printing plate capable of being impregnated by an asphaltum ink-selective composition having ink-receiving portions of hardened asphaltum base material embedded in and penetrating said plate. 18. A planographic printing plate having a grained surface to take water and capable of being impregnated by an asphaltum ink-selective composition and ink-receiving portions of hardened bituminous material penetrating the plate.

THOMAS ERNEST RICHARDS. 135